

J. B. Fuller  
Wood Grinder

№ 41,813. Patented Mar. 1, 1864.



*Witnesses.*

Thos. G. Harwood

### *Inventor.*

Chas. H. Smith

Tim B. Fuller

# UNITED STATES PATENT OFFICE.

JIM. B. FULLER, OF CLAREMONT, NEW HAMPSHIRE, ASSIGNOR TO HIMSELF  
AND JAMES P. UPHAM, OF SAME PLACE.

## IMPROVEMENT IN DISINTEGRATING AND SEPARATING FIBERS OF HEMP, FLAX, &c.

Specification forming part of Letters Patent No. **41 813**, dated March 1, 1864.

*To all whom it may concern:*

Be it known that I, JIM. B. FULLER, of Claremont, in the county of Sullivan and State of New Hampshire, have invented, made, and applied to use a certain new and useful method of separating the fibers of hemp, flax, and similar materials; and I do hereby declare the following to be a full, clear, and exact description of the said invention, reference being had to the annexed drawing, making part of this specification, wherein I have represented a vertical section of an apparatus made use of in carrying out my said method.

In the separation of the fibrous from the woody portions of flax, hemp, &c., it has been usual to ret the same, in order that the gummy matters that cause the fiber to adhere to the stalk may be destroyed, and then said material has been dried so that the woody portions could be easily broken and shaken out of the hanks of the fiber. The disadvantages of these operations are well known, for the retting process makes the fibers more difficult to bleach, and great trouble is still experienced in separating the ultimate fibers of the flax or hemp, because they are so fine and retained together by gummy and silicious matters between the fibers.

The nature of my said invention consists, first, in softening the woody portions of flax, hemp, &c., by steam or hot water under pressure in connection with a pressing operation that acts lengthwise of the fiber to expel a portion of the resinous and foreign matter, (that has been softened and dissolved by said heat and moisture,) split open the stalk, and press the woody portions and fibers together without pulling apart or breaking the fiber. This operation causes the removal to a large extent of the coloring-matter in the green stalk, also the softening and removal of the gums and silicious matter, and the prying apart and separation of the fibers by the woody particles pressed in between them.

The second part of my process consists in rubbing the fibers between suitable moving or rubbing surfaces while in a softened state in the presence of sufficient heat and moisture to cause the separation of the woody particles from the fiber and the separation of the fiber itself to the necessary degree of fineness; and in this connection I employ superheated

steam, whereby I obtain the temperature necessary for the complete dissolving of the gummy and silicious matters at the atmospheric pressure; and I wash the fiber for conveying away the fine woody particles and the resinous and silicious matter either during the use of superheated steam or immediately following the same. I prefer to wash the fiber with hot water, but cold may be employed, because the woody particles rubbed up so finely produce a complete separation of the fiber to its ultimate fineness, or nearly so, and prevent such fibers adhering to each other if cooled.

In the drawing, *a* is a curing-vessel of suitable size and shape. I prefer that it be formed with two parallel sides at a distance apart corresponding to the length of stalk introduced, in order that said stalks may be introduced at right angles to the plane of the section represented. *b* is a man-hole plate or cover provided for closing this curing-vessel after the charge has been introduced. The vessel *a* is formed with an inclined side, whereby the contents may be directed to the long opening or channel *c* that descends to the rollers *d* and *e*. These rollers *d* and *e* are of different sizes, or driven by different sized gears, in order that the surfaces may move at different velocities; and *f* is a fork parallel with the axis of these rollers—that is, moved up and down the channel *c* by a rod, *l*, or other device operated on by suitable mechanism. The rollers *d* and *e* are also driven by suitable mechanism, and are to be incased and provided with springs or weighted levers, so that they will yield to obstructions.

*g* is a pipe for the admission of steam, and *h* is a pipe for the admission of water, both being provided with gates or cocks to regulate the amount supplied.

The operation of this part of the apparatus is as follows: The stock of flax, hemp, or similar material is to be packed into the vessel *a*, as before described, and, if the rollers *d* *e* are sufficiently tight to retain water introduced into the vessel and prevent its leaking away between them, that may be depended upon, otherwise a valve or gate may be introduced in the channel *c*. Steam is to be introduced with water into this vessel *a* under the necessary pressure and heat, and for the period of time required for thoroughly softening the

gums and woody portion of the said material. The rollers *d* and *e* and fork *f* are then set in motion, and the stalks or vegetable material supplied to and squeezed by the rollers *d* *e*, and the fiber going through said rollers nearly parallel to the axes of said rollers is not injured by the pressure, and the woody portion is laid open by said rollers in consequence of one traveling faster than the other and producing a rubbing motion, and the softened and dissolved gums, coloring and silicious matter, are to a considerable extent squeezed onto and removed by the rollers; and this operation may be repeated, or more than one pair of rollers be employed, either with or without hot water or steam applied to the fiber between such pairs of rollers.

The rubbing operation next performed is effected by two corrugated surfaces, *i* and *k*, which may both reciprocate; but I have shown one stationary and forming the top of a steam-chest, *l*, and provided with perforations, whereby steam is allowed to escape and come into direct contact with the fiber while being rubbed between the surfaces *i* and *k*. *m* is a connecting-rod, by means of which *k* can be reciprocated by competent mechanism.

*n n* are bars resting upon the upper surface of the rubber *k*, and *o o* are springs applied to the same to keep the rubber *k* to the rubber *i*. Spring-rollers might be substituted for these bars and perform the same office. The rubber *k* may be hinged at *p* in order that the material may be more easily entered between said surfaces, and the corrugations in such surfaces should be made as shown, in order to cause the material to progress regularly through the machine.

The softened fibrous material is passed in between these rubbing-surfaces with the fibers parallel or nearly so to the corrugations, and the action to which it is exposed between these two surfaces rubs the fibers apart without breaking, injuring, or entangling them, and the woody particles present aid in this operation.

The steam admitted into the chest *l* and

passing upon the fiber under treatment maintains the heat and moisture necessary for a perfect separation of the fibers, and if desired water may be supplied in a similar manner for washing away the fine woody particles or other foreign matter, and squeezing-rollers may be employed at the end of the surfaces where the fiber is worked out in order that the same may be delivered as dry as possible.

The use of superheated steam with many character of fibers is preferable, as operating more quickly than steam at a lower temperature on the silicious and resinous materials. In all cases care must be taken that the steam admitted in jets through the rubbing-surfaces is of the temperature required for acting on the material to the best advantage, and, in order to regulate this temperature, the steam may be admitted from a boiler at a given pressure, or be passed through a coiled pipe in a furnace to superheat said steam; or steam from both such sources may commingle in regulated quantities in the chest *l*.

What I claim, and desire to secure by Letters Patent, is—

1. Separating the gummy and silicious substances from vegetable fiber when softened by heat and moisture by pressing out such dissolved and watery substances by rollers or other suitable mechanism acting lengthwise of the fiber, substantially as specified.
2. Subjecting the vegetable fiber when in a softened state to the action of rollers whose surfaces move at different velocities, for the purposes and substantially as specified.
3. The application to the fibers of flax, hemp, or other substances while being rubbed for their separation of jets of steam of the required temperature, for the purposes and substantially as specified.

Dated December 26, 1863.

JIM. B. FULLER.

Witnesses:

LEMUEL W. SERRELL,  
THOS. GEO. HAROLD.